# EUROPEAN PATENT SPECIFICATION

(11) **EP 3 775 305 B1**
(45) Date of publication and mention of the grant of the patent: **28.06.2023**
(21) Application number: 19726481.5
(22) Date of filing: 12.04.2019
(51) Int. Cl.: C22C 9/00, C22F 1/08, A44C 27/00

(54) **TARNISHING RESISTANT COPPER GOLD ALLOY, IN PARTICULAR 9K, AND METHOD FOR PRODUCTION THEREOF**
ANLAUFBESTÄNDIGE KUPFER-GOLD-LEGIERUNG, INSBESONDERE 9K, UND VERFAHREN ZUR HERSTELLUNG DAVON
ALLIAGE DE CUIVRE ET D'OR, EN PARTICULIER 9K, RÉSISTANT AU TERNISSEMENT, ET SON PROCÉDÉ DE PRODUCTION

(30) Priority: 12.04.2018 CH 4642018
(43) Date of publication of application: 17.02.2021
(73) Proprietor: Argor-Heraeus S.A., 6850 Mendrisio (CH)
(72) Inventor: ARNABOLDI, Sergio, 23867 Suello (IT); ROSSINI, Marta, 6815 Melide (CH); NAUER, Marco, 6834 Morbio Inferiore (CH)
(74) Representative: PGA S.p.A., Milano, Succursale di Lugano
(86) International application number: PCT/IB2019/053023
(87) International publication number: WO 2019/198042

(56) References cited:
- JP-A- 2002 294 361
- KR-A- 20140 001 017
- US-A- 4 527 998
- US-A1- 2008 243 244
- BOYARSHINOVA T S ET AL: "Structure of ordered Au-Cu-Pd alloys", CVETNYE METALLY (TSVETNYE METALLY), MOSKVA : GOS. OB'EDINNOE NAUÃ NO-TECHNIÃ ESKOE IZDAT, RU, no. 12, 1 January 2001 (2001-01-01), pages 47-50, XP009171869, ISSN: 0372-2929
- SUKHANOV ET AL: "Order-disorder transition temperature change in decomposing ternary copper alloys", FIZIKA METALLOV I METALLOVEDENIE (1990), IZDATEL'STVO NAUKA, RU, vol. 75, no. 4, 1 January 1993 (1993-01-01), pages 89-95, XP009188841, ISSN: 0015-3230

## Description

### Field of the invention

The present invention refers to the field of Gold alloys and in particular refers to a Copper Gold alloy with Gold title substantially equal to 9 carats (9K).

The present invention also refers to a method for the production of a Copper Gold alloy.

The Copper Gold alloy and the method for the production of Copper Gold alloys according to the invention are an alloy and a method for the production of Copper Gold alloys for jewellery and watchmaking applications respectively.

### Background art

In the field of the jewellery and watchmaking, Gold is not used in pure form, since it is too ductile. For jewellery and watchmaking applications are typically used Gold alloys for jewellery or watchmaking, characterized by a higher hardness with respect to the Gold in pure form and/or with respect to low hardness or high ductility Gold alloys.

It is known that, generally, Gold alloys can undergo over time unwanted color alterations, following interactions with aggressive environments. These interactions bring to the creation of thin layers of reaction products, which staying adherent to the alloy surface, cause an alteration of the color and of the gloss (document "Observations of onset of sulfide tarnish on gold-base alloys"; JPD, 1971, Vol. 25, issue 6, pag. 629-637).

Environments able to promote color alterations of Gold alloys are various and are linked to their applications.

Colors for Gold alloys can be uniquely measured in the CIELAB 1976 color space, which defines a color on the basis of a first L* parameter, a second a* parameter and a third b* parameter, wherein the first L* parameter identifies the brightness and adopts values comprised between 0 (black) and 100 (white) whereas the second a* parameter and the third b* parameter represent chromaticity parameters. In particular, in CIELAB 1976 color chart, the achromatic scale of greys is detected by points wherein a*=b*=0; positive values for the second parameter a* indicate a color tending the more to red as the higher the value of the second parameter is; negative values for the second parameter a* indicate a color tending the more to green as the value of the second parameter a* is a high absolute value, although negative; positive values for the third parameter b* indicate a color tending the more to yellow as the higher the value of the third parameter is; negative values for the third parameter b* indicate a color tending the more to blue as the value of the third parameter b* is a high absolute value, although negative. Furthermore, it is possible to transform the second a* parameter and the third b* parameter in polar parameters as defined: ${C}_{ab} * = \sqrt{\left(a{∗}^{2}+b{∗}^{2}\right)}$ ${h}_{ab ∗} = {tan}^{- 1} \left(\frac{b ∗}{a ∗}\right)$ The C_{ab}* parameter is defined as "chroma"; the higher the value of C_{ab}* parameter is, the higher is the color saturation; the lower the value of C_{ab}* parameter is, the lower is the color saturation, that will tend to the grey scale. To the knowledge of the Applicant, alloys with a Gold content higher than 750‰, which can be used as such as white or grey Gold alloys and do not require surface rhodium plating, arbitrarily show C_{ab}* values <8. The parameter *h_{ab}** identifies on the other hand the tonality of the color.

In particular, the ISO DIS 8654:2017 standard defines seven color designations as for the Gold alloys for jewellery. In particular, these alloys are defined according to the following table, wherein the color is defined on a standard reference specified between 0N and 6N.

**Table 1**

| Color | Designation |
|---|---|
| 0N | Yellow-green |
| 1N | Dark yellow |
| 2N | Light yellow |
| 3N | Yellow |
| 4N | Pink |
| 5N | Red |
| 6N | Dark red |

For measuring the color of a Gold alloy, in particular, the ISO DIS 8654 standard specifies that the measuring instrument must comply with the CIE N° 15 publication.

The ISO DIS 8654:2017 standard also shows the nominal values L*, a*, b* as trichromatic coordinates for alloys of 0N-6N standard color, including the tolerances. Hereinafter is specified an abstract of the standard wherein are defined the chromatic limits of the alloys defined by the ISO DIS 8654:2017 standard as pink/red.

**Table 2**

| Color | Trichromatic coordinates (2° observer) | | | | | |
|---|---|---|---|---|---|---|
| | Nominal values | | | Tolerances | | |
| | L* | a* | b* | L* [MAX/ Min] | a* | b* |
| 4N | 88.9 | 6.13 | 21.23 | 90.6 | 7.48 | 22.45 |
| | | | | | 6.63 | 19.44 |
| | | | | 87.1 | 4.89 | 19.98 |
| | | | | | 5.48 | 23.06 |
| 5N | 87.7 | 8.32 | 18.58 | 89.4 | 9.74 | 19.55 |
| | | | | | 8.62 | 16.97 |
| | | | | 85.9 | 6.96 | 17.55 |
| | | | | | 7.89 | 20.19 |
| 6N | 86.3 | 10.13 | 15.57 | 88.1 | 11.65 | 16.44 |
| | | | | | 10.14 | 14.06 |
| | | | | 84.4 | 8.70 | 14.65 |
| | | | | | 9.99 | 17.12 |

In relation to the preceding table, it is then possible to obtain, within the CIELAB 1976 color space, a plurality of areas each of which represents the color spaces within which it is possible to assert that an alloy shows a 0N...6N color and more specifically a 5N-6N color. These areas are represented in details in figure 1.

The ISO DIS 8654:2017 standard also proposes chemical compositions recommended for each of the 0N-6N alloys. In particular, for pink/red alloys, the compositions are the ones specified in the table:

**Table 3**

| Color | Chemical composition - % by weight | | |
|---|---|---|---|
| | Au | Ag | Cu |
| 4N | 75.0 | 8.5 - 9.5 | Remaining part |
| 5N | 75.0 | 4.5 - 5.5 | |
| 6N | 75.0 | 0 - 1.0 | |

The Applicant has noted that the pink/red Gold alloys of known type show a substantial color instability, in particular when exposed to environments wherein there are chlorides or sulphides.

Variations of the color of a Gold alloy according to the color as defined on the CIE 1976 color chart and specified by the E=f (L*, a*, b*) coordinate, defined:
- ${L}_{0}^{*}$ as first parameter in original conditions, at time t₀=0;
- ${a}_{0}^{*}$ as second parameter in original conditions, at time t₀=0;
- ${b}_{0}^{*}$ as third parameter in original conditions, at time t₀=0;
are defined in the following equation: $ΔE \left(L*,a*,b*\right) = \sqrt{{\left(L*-{L}_{0}^{*}\right)}^{2} + {\left(a*-{a}_{0}^{*}\right)}^{2} + {\left(b*-{b}_{0}^{*}\right)}^{2}}$

It has also been noted that the human eye of a technician expert in precious materials is able to detect color variations ΔE (L*, a*, b*) >1.

In particular, the Applicant has noted that the 5N ISO DIS 8654:2017 Gold alloy in the formulation that uses the minimum reference value as for the content of Silver exposed to vapors of thioacetamide for 150 hours (according to the UNI EN ISO 4538:1998 standard), shows a variation of color ΔE (L*, a*, b*) equal to 5.6; when exposed to the action of an aqueous solution 50g/liter of sodium chloride (NaCl) at 35°C for 175 hours, the 5N Gold alloy shows a variation of color ΔE (L*, a*, b*) equal to 3.6.

There are also known jewellery alloys, comprising Gold with a title equal to or substantially equal to 9K. These Gold alloys are typically used to make jewels of value lower than those made with 18K or higher Gold alloys. In particular, among the alloys including Gold with a title equal to or substantially equal to 9K, there are known alloys containing Copper, suitable to appear with a pink or red color, according to a growing percentage of Copper in the alloy.

In the alloys including Gold with title equal to or substantially equal to 9K, it is known that the presence of Copper has the drawback of being rather prone to vary color especially when the object of jewelry is worn and exposed to human sweating and/or saline environment. The same alloys, including Gold with a title equal to or substantially equal to 9K are known to have significant color variation even just after exposure to air.

For this reason, typically jewellery items made from alloys including Gold with a title equal to or substantially equal to 9K, in particular when including Copper, are covered with a plating with Gold alloys with a title significantly higher than 9K, typically for example 16K or 18K. This plating has some further drawbacks. A first drawback derives from the fact that it is difficult to realize a plating whose color is perfectly superimposable to that of the basic alloy with which the object of jewellery is made.

Furthermore, the plating of a jewellery item with high title Gold alloys is expensive, and significantly contributes to the increase in the production cost of the item not only because of the cost of the high title Gold alloy, but also because of the further necessary processing on the jewellery item, which incidentally for shapes of jewellery items of considerable complexity, may not be insignificant.

Finally, the plating, representing the surface layer of the item, is the portion the most subject to wear or anyhow removal; with the removal of the plating, the item of jewelry may have exposed portions of alloy with Gold title equal to or substantially equal to 9K, which - exposed to chemically aggressive environments - may have different color than the portions that vice versa still carry the plating alloy.

KR20140001017A discloses an 8 karat gold alloy having discoloration resistance and various colors. An embodiment of this document discloses a copper gold alloy with the following formulation: 33.3% Au, 6.7% Ag, 51,9% Cu, 1,5% Pd, 0,06 % Nd.

US 2008/0243244 A1 discloses a metallic endoprosthesis compatible with magnetic resonance. An example of composition used for the endoprosthesis is: 35% Au, 54.4% Cu, 2.2% Pt, 1% Pd, 6.7% Ag, 0.6% Sn, 0.05% Ir.

Examples of Au-Cu-Pd alloys are disclosed in Boyarshinova T.S. et al. « Structure of Ordered Au-Cu-Pd alloys », Cvetnye Metally (Tsvetnye Metally) Moskva: GOS. OB'EDINNOE NAUA NO-TECHNIA ESKOE Izdat, RU, no 12, 1 January 2001, pp.47-50 (ISSN : 0372-2929).The purpose of the present invention is therefore to describe a Gold alloy, particularly for jewelry and watchmaking, with a Gold title equal to or substantially equal to 9K, which solves the above described drawbacks, in particular being not very prone to turn color when exposed to environments with air, Thioacetamide or NaCl in solution.

The purpose of the present invention is also to describe a method of production of an alloy containing Gold with a title equal to or substantially equal to 9K, which solves the above described drawbacks.

The purpose of the present invention is finally to describe an item of jewelry or part of an item for jewelry, made with the alloy object of the invention, which does not show the above described drawbacks.

### Summary

These and other purposes are obtained by the alloy and by the method of production thereof described in the following aspects. The following aspects may be combined with each other and/or with portions of the description or claims. Where dependencies are indicated, they are described on a preferred and non-limiting basis.

The invention is defined by claim 1. Claim 1 constitutes a first aspect of the disclosure.

Optionally and not limitedly, the sum of Palladium and Iron is equal to 30‰ by weight.

According to the purposes of this invention, as "jewellery alloy" is intended an alloy, in particular a Copper Gold alloy, in which there are no materials toxic to humans and the formulation of which is suitable for, specifically designed for, making jewels, or parts thereof.

According to a 2nd non-limiting aspect, the alloy according to the first aspect is a Copper Gold alloy characterized by a dark red color. According to the present invention, as "dark red" is intended a color that, arbitrarily, on the a*, b* color plan according to the CIE 1976 color chart, is not comprised in the spaces defined by the ISO DIS 8654:2017 standard and is enclosed in a polygon at least defined by the following points:

**Table 4**

| Color | Trichromatic coordinates (2° observer) | | | | | |
|---|---|---|---|---|---|---|
| | Nominal values | | | Tolerances | | |
| | L* | a* | b* | L* [MAX/ Min] | a * | b* |
| dark red | 84.5 | 10 | 12 | 86.3 | 8.2 | 10.6 |
| | | | | | 10 | 10.2 |
| | | | | 82.8 | 11.2 | 13 |
| | | | | | 9.71 | 13.55 |

According to a 3rd non-limiting aspect, the alloy according to the first or second aspect is a tarnishing resistant alloy.

According to a 4th non-limiting aspect, the alloy depending on one or more of the preceding aspects, comprises Palladium in an amount of 8‰, preferably 10‰ by weight, and 32‰, more preferably 30‰ by weight.

According to a 5th non-limiting aspect, the alloy according to one or more of the preceding aspects, comprises also Iron in an amount of 2‰ by weight to 25‰ by weight, more preferably of 5‰ by weight to 20‰ by weight.

According to a 6th non-limiting aspect, the alloy according to one or more of the preceding aspects is a ternary or quaternary alloy, and the sum of the amounts of Gold, Copper and Palladium is at least equal to 900‰ by weight.

According to the present invention, as ternary or quaternary Gold alloy is intended an alloy wherein there are 3 or 4 components respectively, the amount of which is not negligible.

According to a 7th non-limiting aspect, the alloy according to the 6th aspect shows a sum of the amounts of Gold, Copper and Palladium at least equal to 960‰ by weight, preferably 970‰ by weight.

According to a 8th non-limiting aspect, which does not form part of the present invention, the alloy according to the 6th aspect comprises also Silver in an amount lower than 100‰ by weight, and/or Zinc in an amount lower than 100%o by weight or Silver and Zinc the sum of respective amounts by weight is lower than 100‰.

According to a 9th non-limiting aspect, the alloy according to one of the aspects from 1st to 7th, comprises Palladium in an amount of 15‰ by weight to 25‰ by weight, preferably between 18‰ by weight to 22‰ by weight, more preferably substantially equal to 20‰ by weight.

According to a 10th non-limiting aspect, in the alloy according to one of the aspects from 1st to 7th, when depending on the 5th aspect, the sum of the amounts of Palladium and Iron is equal to 30‰ by weight.

According to a 11th non-limiting aspect, in the alloy according to one or more of the preceding aspects, the Gold is present in an amount of 365‰ by weight to 385‰ by weight and Copper is present in an amount of 594‰ by weight to 614‰ by weight and Palladium is of 15‰ to 25‰ by weight, more in particular of 18‰ to 22‰ by weight.

In particular, according to a 12th non-limiting aspect, the alloy according to the 11th aspect, is free from Iron.

According to a 13th non-limiting aspect, the alloy subject of the invention is an alloy whose color on the CIELAB1976 color chart shows a coordinate a* > 8.2 and a coordinate b*<13.5.

According to a 14th non-limiting aspect, said Copper Gold alloy for jewellery is an alloy characterized by the absence of Vanadium, and other materials capable to create carbides and oxides, in particular free from Magnesium, Silicon, Titanium, Tungsten, Molybdenum, Niobium, Tantalum, Zirconium, Yttrium, Germanium.

According to a 15th non-limiting aspect, the Copper Gold alloy for jewellery is an alloy free from Nickel, Cobalt, Arsenic and Cadmium. Thanks to this aspect, the alloy is a Copper Gold alloy compatible with being worn or wearable by subjects whose allergic tolerance is significantly low.

A further object of the invention is the method according to claim 8. Such method constitutes a 16th aspect.

According to a 17th non-limiting aspect, depending on the preceding 16th aspect, said step comprises mixing in particular Palladium in an amount of 8‰, preferably 10‰, to 32‰, preferably 30‰ by weight.

According to a 18th non-limiting aspect, the alloy according to one or more of the preceding 16th-17th aspects, comprises in particular mixing, in addition to the preceding elements, also Iron in an amount of 2‰ by weight and 25‰ by weight, more preferably of 5‰ by weight and 20‰ by weight.

According to a 19th non-limiting aspect, in the alloy according to one or more of the preceding aspects from 16th to 18th, the sum of the amounts of Gold, Copper and Palladium is at least equal to 900‰ by weight.

According to a 20th non-limiting aspect, the step comprises the mixing of Gold, Copper and Palladium in an amount at least equal to 960‰ by weight, more preferably 970‰ by weight.

According to a 21st non-limiting aspect, which does not form part of the present invention, the alloy according to the 19th aspect comprises the mixing of Silver in an amount lower than 100‰ by weight, and/or Zinc in an amount lower than 100%o by weight or Silver and Zinc the sum of respective amounts by weight is lower than 100‰.

According to a 22nd non-limiting aspect, according to one of the aspects from 16th to 21st, said step comprises the mixing of Palladium in an amount of 15‰ by weight to 25‰ by weight, preferably between 18‰ by weight to 22‰ by weight, more preferably substantially equal to 20‰ by weight.

According to a 23rd non-limiting aspect, when depending on the 18th aspect, the sum of the amounts of Palladium and Iron is equal to 30‰ by weight.

According to a 24th non-limiting aspect, depending on one or more of the preceding aspects from 16th to 23rd, the Gold is mixed in particular in an amount of 365‰ by weight to 385‰ by weight and Copper is present between 594‰ by weight to 614‰ by weight and Palladium is of 15‰ to 25‰ by weight, preferably between 18‰ to 22‰ by weight.

According to a 25th non-limiting aspect, said homogenization is a discontinuous melting, comprising a step of casting wherein the melted material is cast in a refractory mold or refractory or metallic ingot and wherein said melted alloy is an alloy characterized by the absence of Vanadium, and other elements capable to create carbides or oxides, in particular free from Magnesium, Silicon, Titanium, Tungsten, Molybdenum, Niobium, Tantalum, Zirconium, Yttrium, Germanium. The absence of said carbides or oxides makes the Copper Gold alloy suitable for applications of jewelry and watchmaking where polishing or diamond polishing of finished items is required.

According to a 26th non-limiting aspect, during said melting, the melting pot is subject to a gas controlled atmosphere and in particular is subject, at least temporarily, to vacuum condition.

According to a 27th non-limiting aspect, during said casting step, said melting pot is subject to a controlled atmosphere, to pressures lower than the environmental one.

According to a 28th non-limiting aspect, said controlled atmosphere is or comprises an inert gas, preferably argon and/or said pressure is a pressure lower than 800mbar, preferably lower than 700mbar.

According to a 29th non-limiting aspect, said gas is a reducing gas, preferably a hydrogen-nitrogen mixture and/or said pressure is a pressure lower than 800mbar, preferably lower than 700mbar.

According to a 30th non-limiting aspect, said melting is a continuous melting, comprising a step of melting and homogenization in a graphite pot and a subsequent melting step wherein the melted alloy is cast in a die realized in graphite and wherein said alloy is an alloy of metals without chemical affinity to graphite and more specifically, in particular at least free from Vanadium, Magnesium, Silicon, Titanium, Tungsten, Molybdenum, Niobium, Tantalum, Zirconium, Yttrium, Germanium.

The absence of elements with chemical affinity to graphite allows an excellent flow of the melted alloy within the die and facilitates the extraction thereof after solidification. On the contrary, the presence of elements with chemical affinity to graphite, causes a gripping effect of the alloy to the die, preventing the extraction. Furthermore, the absence of carbides and oxides makes the Copper Gold alloy suitable for applications of jewelry and watchmaking where polishing or diamond polishing of finished items is required.

According to a 31st non-limiting aspect, after the continuous or discontinuous melting, said alloy is subject to a cooling step followed by one or more hot or cold plastic deformation steps and one or more thermal treatments.

According to a 32nd aspect, it is also object of the present invention an item of jewelry according to claim 14.

According to a 33rd aspect, depending on the preceding aspect, said item of jewellery comprises a jewel or a watch or a watch bracelet or a movement or part of a mechanical movement for watches.

According to a 34th aspect, depending on the preceding aspect, said watch or mechanical movement for watches are configured for being respectively worn or installed in wristwatches.

According to a 35th aspect, that can be combined with one or more of the preceding aspects, the Copper Gold alloy is free from secondary phases, and/or is a homogeneous alloy, and/or is a crystalline alloy, optionally 100% crystalline.

According to the present invention, as "free from secondary phases" or "free from second phases" is intended an alloy free from elements that can generate said second phases, in particular in a proceeding of melting and subsequent solidification without other thermal treatments; second phases that create in the liquid phase and remain downstream of the alloy solidification, are harmful second phases, for example carbides and/or oxides that during the polishing step are visible at naked eye on the surface of the polished item, and that then prevent to obtain items of high surface quality, compatible with the needs required in the high jewellery field. It is possible to expose the alloy to thermal treatment processes, able to give it a hardening, so that due to precipitation subtle precipitates can be present, as results of said thermal treatment; in this case these are precipitates that prevent from the movement of displacement by increasing the mechanical properties in the material, and contrasting the incidence of deformations in the items realized with the present alloys.

### Description of drawings

The invention is hereinafter described in preferred and non-limiting embodiments, whose description is associated to the attached figures wherein:
- Figure 1 shows a portion of CIELAB 1976 color space according to the coordinates L*, a*, b* wherein it has been detected an area corresponding to color intervals or tolerances admissible for Gold alloys according to the 5N and 6N ISO DIS 8654:2017 standard and wherein it is shown the typical color position for alloys object of the present invention;
- Figure 2 shows color variation charts according to the time of exposure to 50g/L of Sodium Chloride solutions for alloys object of the present invention, in relation to the color variation gained by the 5N 18K alloy according to the ISO composition used as reference sample and in relation to the color variation of a reference Gold, Silver and Copper red ternary 9K alloy (LRS 362, defined hereinafter in Tab. 6);
- Figure 3 shows a color variation chart according to the time of exposure to Thioacetamide solutions according to UNI EN ISO 4538 for part of the alloys object of the present invention, in relation to the color variation gained by the 5N 18K alloy according to the ISO composition used as reference sample and in relation to the color variation of a reference Gold, Silver and Copper red ternary 9K alloy (LRS 362, defined hereinafter in Tab. 6);
- Figure 4 shows a curve of variation of the color variation rate of various alloys object of the present invention when exposed for a determined time period to Thioacetamide according to the content of Palladium;
- Figure 5 shows a curve of variation of the color variation rate of various alloys object of the present invention when exposed for a determined time period to NaCl aqueous solution according to the content of Palladium.

### Detailed description

It is an object of the present invention to provide a family of Copper Gold alloys, in particular for jewellery, with Gold title comprised between 8K and 10K, that have tarnishing resistance characteristics.

The alloys that are described in the present invention have been tested in terms of resistance to color variation (tarnishing) in environments comprising Thioacetamide and NaCl solutions (sodium chloride). In this description, any reference to tests carried out in an environment comprising Thioacetamide is made according to the indications of the UNI EN ISO4538:1998 standard. In order to carry out the tests, according to the present invention, the samples are exposed to vapours of Thioacetamide CH₃CSNH₂ in an atmosphere with relative humidity of 75% kept through the presence of a saturated solution of sodium acetate trihydrate CH₃COONa·3H₂O in a test chamber with a capacity comprised between 2 and 20 litres and wherein all the materials used for the construction of the chamber itself are resistant to volatile sulphides and do not emit any gas or vapour capable of influencing the results of the test.

With regard to the assessment of the resistance to corrosion and color variation in environments characterized by the presence of Sodium Chloride solutions, the tests have been carried out by immersing the samples of a Copper Gold alloy in a 50g/L NaCl solution at neutral pH, thermostated at 35°C.

In order to obtain tarnishing resistance properties, in particular in environments comprising solutions of Thioacetamide and NaCl according to the above described standards and also to obtain a Copper Gold alloy whose color, measured according to the ISO DIS 8654:2017 standard is contained in the color space defined as "dark red", the Applicant has conceived a family of Copper Gold alloys according to claim 1.

According to the present invention, with "tarnishing" is intended a surface corrosion of the Copper Gold alloy that causes a variation in the alloy color.

The family of Copper Gold alloys object of the invention comprises at least ternary alloys, and in particular ternary or quaternary alloys. Therefore, the number of elements that are included in a not insignificant amount in the family of Copper Gold alloys object of the invention is at least equal to 3 and, preferably, not higher than 4.

The Applicant has carried out various experiments for assessing the resistance to tarnishing and the so obtained color of the alloys, and in particular has carried out experiments on the specific embodiments indicated in the following table:

**Table 5**

| **Nominal composition % by weight]** | | | | | | |
|---|---|---|---|---|---|---|
| **LRS** | **Au** | **Ag** | **Cu** | **Pd** | **Fe** | **Total** |
| **479** | 375.5 | | 609.5 | 15.0 | | 1000 |
| **480** | 375.5 | | 614.5 | 10.0 | | 1000 |
| **495** | 375.5 | | 594.5 | 25.0 | 5 | 1000 |
| **496** | 375.5 | | 594.5 | 20.0 | 10 | 1000 |
| **497** | 375.5 | | 604.5 | 20.0 | | 1000 |
| **498** | 375.5 | | 584.5 | 20.0 | 20 | 1000 |
| **499** | 375.5 | | 599.5 | 25.0 | | 1000 |
| **500** | 375.5 | | 594.5 | 30.0 | | 1000 |

In the above table, as in the other tables of the present description, where the boxes are empty, it is intended a zero percentage of the relevant element.

The alloys according to the preceding formulations are preferred and non-limiting examples of Copper Gold alloy for jewellery with a title equal to or substantially equal to 9K. The tarnishing resistance tests carried out by the Applicant and reported below have been carried out with respect to a reference alloy, in particular a reference ternary alloy comprising Gold, Copper and Silver, whose composition is the following.

**Table 6**

| **Reference alloy nominal composition [% by weight]** | | | | | | |
|---|---|---|---|---|---|---|
| **LRS** | **Au** | **Ag** | **Cu** | **Pd** | **Fe** | **Total** |
| **362** | 375.5 | 99 | 525.5 | | | 1000 |

The LRS 362 alloy used as reference test does not have a "dark red" color, but a significantly different color, which lies within the tolerances for alloys whose color is compatible with 6N ISO.

The alloys according to the family generally described as the object of the invention and, consequently, the specific realizations described in table 5 are realizations characterized by the absence of Silver. Silver is known to be an element that in these alloys helps to increase the hardness. As an example, the 362 alloy used as reference test, in the absence of work hardening, has a hardness according to HV5 equal to 139, which becomes equal to 185 with 25% work hardening, equal to 210 with 50% work hardening and equal to 245 with 75% work hardening. In particular, for the alloys listed in Table 5, it has been searched an alternative solution to Silver, which could also help to keep the hardness of the specific formulation of alloy suitable for jewellery applications, such as to make the formulation "for jewellery" as defined in the preceding definition, avoiding the trend to tarnishing that Silver helps to bring for alloys where it is contained.

The following table shows the hardnesses obtained for the specific alloy formulations according to the present invention, as well as for the LRS 362 alloy used as reference test.

**Table 7**

| **HV5** | **% work hardening** | | | |
|---|---|---|---|---|
| **LRS** | **0** | **25** | **50** | **75** |
| **362** | **139** | **185** | **210** | **245** |
| **479** | **115** | **179** | **210** | **220** |
| **480** | **111** | **178** | **189** | **208** |
| **495** | **121** | **174** | **185** | **229** |
| **496** | **138** | **175** | **192** | **250** |
| **497** | **105** | **171** | **187** | **210** |
| **498** | **155** | **181** | **213** | **244** |
| **499** | **100** | **120** | **106** | **220** |
| **500** | **105** | **115** | **190** | **225** |

The Applicant has observed that the specific formulations of Copper Gold alloy described in table 7 have hardness, even under conditions of non-work hardening, compatible with that of alloys for jewellery in accordance with the present invention. In particular, the LRS 496 and LRS 498 formulations are respectively the closest to the behavior in terms of hardness possessed by the LRS362 alloy used as reference test (whose alignment in the table is offset for ease of identification), and even better (LRS 498) with respect to the alloy used as reference test. This shows that in order to obtain hardnesses that are also optimal for the processing of jewels that require considerable resistance in terms of hardness, equal to or substantially equal to the hardness of a ternary Gold-Copper-Silver alloy, that however - due to the presence of a significant amount of Silver - is strongly subject to tarnishing - it is possible to introduce into the alloy a quantity equal to at least 30‰ of Palladium and Iron, in which Iron is contained in an amount of at least 10‰. In particular, the Applicant has highlighted that in a 9K quaternary Gold-Copper-Palladium and Iron alloy, having a quantity equal to 40‰ of Palladium and Iron, and in particular having Palladium and Iron in amounts respectively comprised, each one, of 18‰ to 22‰, and more in particular each one in amounts equal to 20‰ allows to obtain alloys whose hardness is substantially higher than the LRS362 reference alloy, at least up to a level of hardening equal to 50%.

The Applicant has observed as it will be better described hereinafter that all the alloys object of the invention and belonging to the above mentioned family, and in particular but non-limiting to the alloys object of table 5 have better performances in Air, Thioacetamide and NaCl solution under the above mentioned conditions, in terms of resistance to color variation, with respect to what can be obtained with the LRS 362 alloy used as reference test. The graphs in Figure 2 and Figure 3 respectively illustrate the evolution of the color of some specific alloy formulations as the number of hours of exposure to NaCl saline solution and Thioacetamide increases, as for the above indicated specifications.

All the alloys according to the invention, and in particular all the specific realizations of the alloys according to table 5 have a better behaviour, both in NaCl solution and in Thioacetamide, with respect to the LRS362 alloy used as reference test. This shows that the elimination of Silver, among other things, is beneficial for reducing the trend of the alloy to turn color when exposed to chemically aggressive environment. In fact, although the alloy used as a reference test has a color that is not compatible with that of the alloys object of the invention, the latter have a significantly lower trend to change color.

In particular, the Applicant has observed that the optimization of the alloy behavior in terms of tarnishing is optimized - in the ranges identified in the preceding family, for Palladium values comprised within the following range: [8‰ - 32‰] by weight, and preferably for Palladium values within the range of [10‰ - 30‰] by weight.

From the tests carried out in NaCl saline solution as above indicated, the Applicant has surprisingly verified that the optimization of the resistance to tarnishing is obtained, for the family as generally above expressed, for Palladium contents in an amount of 15‰ by weight and 25‰ by weight, in particular of 18‰ by weight to 22‰ by weight, and more in particular for Palladium contents substantially equal to 20‰ by weight. In particular, for alloys in which the Gold content is of 365‰ to 385‰ by weight, and in which Copper content is of 594‰ to 614‰ by weight, and in which Palladium content is of 15‰ by weight to 25‰ by weight, and specifically between 18‰ by weight and 22‰ by weight, the Applicant has observed a substantial optimal behavior of performances in NaCl, in particular when Iron content in the alloy is lower than 20‰ and in particular when Iron content is lower than or equal to 10‰. In particular, as shown in the graph in Figure 2, alloys according to the LRS 496 and 497 formulation, respectively with an Iron content equal to 10%o by weight and zero, have an optimized behavior. Surprisingly, the Applicant was able to conceive alloys that, with the above mentioned formulations and in particular with Palladium of 18‰ to 22‰ and Iron in an amount lower than or equal to 10‰, the performances of a 9K alloy are substantially close to that of an alloy according to the 5N ISO standard, which has a significantly higher Gold title, because at 18K. Therefore, it was almost possible to achieve, in terms of tarnishing, the behavior of an 18K alloy with an alloy whose Gold content is significantly lower, being 9K.

The following table describes the color variation characteristics ΔE (L*, a*, b*) according to the exposure time in NaCl saline solution.

**Table 8**

| ***ΔE*** | **Time (h)** | | | | |
|---|---|---|---|---|---|
| | **0** | **2** | **4** | **24** | **48** |
| **5N ISO** | 0.00 | 0.77 | 1.39 | 2.03 | 2.37 |
| **LRS 362 (Ref. ternary)** | 0.00 | 0.28 | 1.86 | 8.62 | 11.79 |
| **LRS 479** | 0.00 | 0.65 | 1.70 | 10.75 | 15.67 |
| **LRS 480** | 0.00 | 0.41 | 2.45 | 18.04 | 24.91 |
| **LRS 495** | 0.00 | 2.90 | 3.40 | 6.70 | 8.12 |
| **LRS 496** | 0.00 | 0.52 | 1.10 | 3.80 | 3.90 |
| **LRS 497** | 0.00 | 0.49 | 0.97 | 3.40 | 3.77 |
| **LRS 498** | 0.00 | 0.87 | 1.00 | 5.12 | 6.47 |
| **LRS 499** | 0.00 | 0.41 | 0.77 | 4.59 | 5.39 |
| **LRS 500** | 0.00 | 0.95 | 2.60 | 4.30 | 5.13 |

From the above indicated table and from the graph of figure 2 it is possible to observe that the specific LRS 479 and 480 formulations have a worse behavior in NaCl than the LRS362 alloy used as reference test. On the other hand, in Thioacetamide according to the above mentioned conditions, the behaviour of the alloys according to the invention, and in particular all the alloys according to the above mentioned specific formulations have a better behaviour than the one of the LRS362 alloy used as reference test, even if they cannot match the performances of the 5N ISO alloy in the same environment due to the lower Gold content.

The following table describes the color variation characteristics ΔE (L*, a*, b*) according to the exposure time in Thioacetamide.

**Table 9**

| | **Time (h)** | | | | |
|---|---|---|---|---|---|
| **ΔE** | **0** | **1** | **2** | **8** | **24** |
| **5N ISO** | 0.00 | 0.76 | 2.12 | 3.12 | 3.73 |
| **LRS 362 (Ref. ternary)** | 0.00 | 0.68 | 1.80 | 5.45 | 16.50 |
| **LRS 479** | 0.00 | 0.38 | 1.94 | 4.46 | 13.67 |
| **LRS 480** | 0.00 | 0.41 | 1.80 | 4.45 | 15.14 |
| **LRS 495** | 0.00 | 0.31 | 1.70 | 4.03 | 10.94 |
| **LRS 496** | 0.00 | 0.52 | 1.35 | 4.01 | 9.60 |
| **LRS 497** | 0.00 | 0.34 | 1.03 | 3.69 | 8.50 |
| **LRS 498** | 0.00 | 0.30 | 0.79 | 3.92 | 13.60 |
| **LRS 499** | 0.00 | 0.38 | 0.99 | 3.78 | 15.29 |
| **LRS 500** | 0.00 | 0.39 | 1.17 | 3.76 | 15.40 |

As it can be seen from the reading of Table 9 in conjunction with Table 5 and the graphs in Figures 3, 4 and 5, the Applicant has surprisingly discovered that the behaviour of ternary or quaternary Gold-Copper-Palladium or Gold-Copper-Palladium and Iron 9K Copper Gold alloys is strongly optimized for Palladium values substantially of 18‰ to 22‰, with an optimization peak (lower ΔE values, and minimum of the curve in the graph of Figures 4 and 5) for an amount of Palladium equal to 20‰, both in Thioacetamide (Figure 4) and in NaCl (Figure 5).

In order to reduce the risk that the inclusion of third-party elements in the preceding alloy family may lead to unpredictable behaviors, the Applicant has observed that the alloy must be preferably ternary or quaternary, with the necessary presence of Palladium and with the sum of the amounts of Gold, Copper and Palladium at least equal to 900‰ by weight..

**Table 10**

| | **2° observer** | | |
|---|---|---|---|
| | **L*** | **a*** | **b*** |
| **LRS 362** | 87.5 | 9.7 | 16.0 |
| **LRS 479** | 85.64 | 10.43 | 12.70 |
| **LRS 480** | 85.89 | 10.72 | 13.00 |
| **LRS 495** | 85.3 | 10.0 | 11.8 |
| **LRS 496** | 85.56 | 9.17 | 11.36 |
| **LRS 497** | 85.28 | 8.94 | 11.23 |
| **LRS 498** | 84.50 | 9.08 | 12.09 |
| **LRS 499** | 83.73 | 10.07 | 12.88 |
| **LRS 500** | 83.16 | 9.69 | 12.50 |

From the preceding Table 10, it is clear that the LRS 362 alloy used as reference test is the only one with a significantly different color with respect to the others, and that it is not "dark red" according to the present invention, since it falls within the tolerance limits defined for alloys whose color complies with the 6N ISO standard.

In particular, all the embodiments specifically identified in Table 5 are specific optimized embodiments taken from a subfamily of alloys in which the sum of the amounts of Gold, Copper and Palladium is at least equal to 960‰ by weight and preferably 970‰ by weight; alloys with this last characteristic have a substantially assimilable behavior in the complex, observing the color variations in air, in Thioacetamide and in NaCl solution.

In particular, and not belonging to the present invention, Iridium is preferably used in alloys containing high Copper contents, because it binds in particular with the latter element; preferably, but non-limiting thereto, if present, Iridium is present in an amount equal to or lower than 0.5‰ by weight. Rarer is the use of Ruthenium and Rhenium, in a sometimes lower amount, but anyway up to 0.5 ‰ by weight. Ruthenium and Rhenium are used in Copper Gold alloys containing Palladium or Zinc in an amount lower or equal to 100‰.

However, it is noted that the use of Iridium and/or Rhenium and/or Ruthenium is subject to the inclusion of these elements in pre-alloys. In fact, it has been observed that these elements, if not pre-alloyed with the material with affinity thereto, but directly introduced into the pot, do not form alloy, thus contributing to a worsening of the characteristics of the alloy. On the other hand, only if used in pre-alloy with Copper (Iridium) or Palladium (Rhenium and Ruthenium), taking care to make the pre-alloy bind with the rest of the elements composing the alloy itself, it is possible to refine the grain.

With the purpose of reducing the risk of formation of carbides during the processing, the Copper Gold alloy for jewellery is preferably characterized by the absence of Vanadium and other materials capable to create carbides and oxides, in particular free from Magnesium, Silicon, Titanium, Tungsten, Molybdenum, Niobium, Tantalum, Zirconium, Yttrium, Germanium.

This alloy is also an alloy free of Nickel, Cobalt, Arsenic and Cadmium. Thanks to this aspect, the alloy is a Copper Gold alloy compatible with being worn or wearable by subjects whose allergic tolerance is significantly low.

It is also object of the invention a process of production of a Copper Gold alloy.

The Copper Gold alloys of the invention are made from pure elements in particular from Gold at 99.99%, Cu at 99.99%, Pd at 99.95%, Fe at 99.99%.

The process of melting of pure elements for the creation of the Copper Gold alloys according to the invention can be in detail a process of discontinuous melting of Gold or a process of continuous melting of Gold. The process of discontinuous melting of Gold is a process in which the mixing is melted and cast into a refractory mold or refractory or metallic ingot mould. In this case the above mentioned elements are melted and cast in a controlled atmosphere. More in particular, the melting operations are carried out only after having preferably conducted at least 3 conditioning cycles of the atmosphere of the melting chamber. This conditioning involves first of all reaching a vacuum level up to pressures lower than 1×10⁻² mbar and a subsequent partial saturation with Argon at 500mbar. During the melting, the Argon pressure is kept at pressure levels between 500mbar and 800mbar. When the complete melting of the pure elements has been reached, a phase of overheating of the mixture takes place, in which the mixture is heated up to a temperature of about 1250°C, and in any case to a temperature above 1200°C, in order to homogenize the chemical composition of the metal bath. During the overheating phase, the pressure value in the melting chamber reaches again a vacuum level lower than 1×10⁻² mbar, useful to eliminate part of the residues produced by the melting of the pure elements.

At this point, in a casting step, the melted material is cast into a mould or ingot mould realized in graphite and the melting chamber is again pressurized with an inert gas, preferably argon, injected at a pressure lower than 800mbar and in particular lower than 700mbar.

After solidification, the bars or casts are extracted from the bracket. When the alloy is solidified, from the mold in graphite are obtained Gold bars or Copper Gold alloy casts which are subjected to quick cooling by means of a step of immersion in water, in order to reduce and possibly avoid solid state phase transformations. In other words, the bars or casts are subjected to a quick cooling phase, preferably but non-limiting in water, in order to avoid phase variations in the solid state.

In a more general embodiment, the production process of the Copper Gold alloy according to the invention comprises, starting from the pure elements according to the above, a mixing step of elements according to the present disclosure, and in particular:
- Gold, in an amount of 330‰ to 420‰ by weight;
- Copper, in an amount of 500‰ to 620‰ by weight;
- Palladium, in an amount of 5‰ to 35‰ by weight;
and a step of introduction of the mixture in a melting pot, and a subsequent melting through heating until melting.

The process of continuous melting is a process in which solidification and extraction of the solidified Gold are continuously carried out from one free end of a Gold bar or cast. In particular, a graphite die is used in the continuous melting process. The use of graphite dies is known, since graphite is a solid lubricant, and typically has low friction between its surfaces and those of the solidified metal, permitting to obtain an easy extraction of the element contained therein without fractures and with the minimum amount of defects present on its surface.

When the inclusion of Iridium, Indium, Ruthenium and Rhenium is present for grain refinement, which does however not form part of the present invention, the production process comprises a step of realizing of a pre-alloy in which said pre-alloy comprises:
a) Iridium pre-alloyed to Copper in the already indicated amounts, or alternatively
b) Rhenium or Ruthenium pre-alloyed to Palladium in the already indicated amounts.

Subsequently, the bars or casts obtained by discontinuous or continuous melting are subject to a step of cold plastic deformation, preferably but non-limiting to flat rolling.

During the flat rolling and more generally during the cold plastic processing steps, the different compositions synthesized according to the previously described melting procedure are deformed by more than 70% and then subjected to a thermal treatment of solubilization at a temperature higher than 680°C, in order to be subsequently cooled.

Particular embodiments of the previously described method include an initial step in which are mixed in particular Palladium in an amount of 8‰, preferably 10‰, and 32‰, more preferably 30‰ by weight and/or, in addition to the preceding elements, also Iron of 2‰ by weight to 25‰ by weight, more preferably between 5‰ by weight to 20‰ by weight.

In a particular embodiment of the method of realization of the Copper Gold alloy, the sum of the amounts of Gold, Copper and Palladium is at least equal to 900‰ by weight, and in particular in an amount at least equal to 960 ‰ by weight, more preferably 970 ‰ by weight.

In case the sum of the amounts of Gold, Copper and Palladium is at least equal to 900 %o, it is possible to carry out a step of addition of Silver in an amount lower than 100%o by weight, and/or Zinc in an amount lower than 100%o by weight or Silver and Zinc of which the sum of respective amounts by weight is lower than 100‰.

In a particular embodiment of the method, it is possible to mix Palladium in an amount of 15‰ by weight to 25‰ by weight, preferably in an amount of 18‰ by weight to 22‰ by weight, more preferably substantially equal to 20‰ by weight, in such a way that, for example, the sum of the amounts of Palladium and Iron is equal to 30‰ by weight.

In a particular embodiment of the method of production of the Copper Gold alloy object of the invention, the Gold is mixed in particular in an amount of 365‰ by weight to 385‰ by weight and Copper is present in an amount of 594‰ by weight to 614‰ by weight and Palladium is present in an amount of 15‰ to 25‰ by weight, preferably in an amount of 18‰ to 22‰ by weight.

The advantages offered by the alloy object of the invention are clear in the light of the above obtained description. The alloys are characterized by a low trend to tarnishing for the environments in which an item of jewellery is typically found to be used, consequently it allows to realize items of jewellery or parts of items for jewellery resistant to tarnishing, in substantially red color as above defined, without the need for subsequent plating with high title Copper Gold alloys. Consequently, the item of jewellery thus created is less expensive and less demanding to be processed as well as characterized by a substantially more uniform color even after wear.

The alloys according to the present disclosure are alloys without secondary phases. In detail, the alloys according to the present disclosure are homogeneous Copper Gold alloys, free from second phases, and in particular free from carbides and/or oxides and/or are crystalline alloys, in particular 100% crystalline. This permits to have a high strength and quality and surface uniformity. In the here described process of production of the Copper Gold alloy, it is possible to expose the alloy to thermal treatment processes, able to give it a hardening, so that due to precipitation can be present subtle precipitates, results of said thermal treatment; in this case these are precipitates that prevent from the movement of displacement by increasing the mechanical properties in the material, and withstand the incidence of deformations in the items realized with the present alloys.

## Claims

1. An alloy, in particular for jewellery, **characterized in that** it consists of:
- Gold, in an amount of 330‰ to 420‰ by weight;
- Copper, in an amount of 500‰ to 620‰ by weight;
- Palladium, in an amount of 5‰ to 35‰ by weight;
and optionally Iron in an amount of 2‰ to 25‰ by weight, preferably of 5‰ to 20‰ by weight.

2. Alloy according to claim 1, **characterized in that** it has a dark red color and/or in that it has a color that, on the CIELAB1976 color chart, has a coordinate a* > 8.2 and a coordinate b*<13.55, wherein the CIELAB1976 color chart defines a color on the basis of a first L* parameter, a second a* parameter and a third b* parameter, the first L* parameter identifying the brightness and adopting values comprised between 0 for black and 100 for white, whereas the second a* parameter and the third b* parameter represent chromaticity parameters, said second a* and third b* parameters being related by the following formulas ${C}_{ab} * = \sqrt{\left(a{∗}^{2}+b{∗}^{2}\right)}$ ${h}_{ab ∗} = {tan}^{- 1} \left(\frac{b ∗}{a ∗}\right)$ wherein C_{ab}* is defined as "chroma" and identifies the color saturation, and wherein *h_{ab∗}* identifies the tonality of the color.

3. Alloy according to any of the preceding claims, wherein Palladium is present in an amount of 8‰, preferably of 10‰ by weight, to 32‰, more preferably to 30‰ by weight.

4. Alloy according to claim 3, wherein Palladium is present in an amount of 15‰ to 25‰ by weight, preferably of 18‰ to 22‰ by weight, more preferably in an amount substantially equal to 20‰ by weight.

5. Alloy according to one or more of the preceding claims, wherein the sum of the amounts of Palladium and Iron is equal to 30‰ by weight.

6. Alloy according to any of the preceding claims, wherein Gold is present in an amount of 365‰ to 385‰ by weight and Copper is present in an amount of 594‰ to 614‰ by weight and Palladium is comprised in an amount of 15‰ to 25‰ by weight, optionally in an amount of 18‰ to 22‰ by weight.

7. Alloy according to any of the preceding claims, **characterized by** the absence of Vanadium, and other metals capable to create carbides and oxides, in particular free from Magnesium, Silicon, Titanium, Tungsten, Molybdenum, Niobium, Tantalum, Zirconium, Yttrium, Germanium, said alloy being also free from Nickel, Cobalt, Arsenic and Cadmium.

8. A method of production of a Copper Gold alloy for jewellery; said method being **characterised in that** it comprises:
a) a step of homogenization of:
- Gold, in an amount of 330‰ to 420‰ by weight;
- Copper, in an amount of 500‰ to 620‰ by weight;
- Palladium, in an amount of 5‰ to 35‰ by weight;
- and optionally Iron in an amount of 2‰ to 25‰ by weight, preferably of 5‰ to 20‰ by weight;
for creating a mixture; and
b) a step of introduction of the mixture in a melting pot, and a subsequent melting through heating until melting.

9. Method according to claim 8, wherein, said homogenization is a discontinuous melting, comprising a step of casting, wherein the melted material is cast in a refractory mold and wherein said melted alloy is an alloy **characterized by** the absence of Vanadium, and other elements capable to create carbides or oxides, in particular free from Magnesium, Silicon, Titanium, Tungsten, Molybdenum, Niobium, Tantalum, Zirconium, Yttrium, Germanium.

10. Method according to claim 9, wherein the melting pot is subject to a gas controlled atmosphere and in particular is subject, at least temporarily, to vacuum condition.

11. Method according to claim 9 or 10, wherein during said casting step, said melting pot is subject to a controlled atmosphere, and to pressures lower than the environmental one and wherein said controlled atmosphere is or comprises an inert gas, preferably argon and/or said pressure is a pressure lower than 800mbar, preferably lower than 700mbar and/or wherein said gas is a reducing gas, preferably a hydrogen-nitrogen mixture.

12. Method according to claim 11, wherein said melting is a continuous melting, comprising a step of melting and homogenization in a graphite pot and a subsequent casting step wherein the melted alloy is casted in a mold realized in graphite and wherein said alloy is an alloy of metals chemically not similar to the graphite and more specifically, in particular at least free from Vanadium, Magnesium, Silicon, Titanium, Tungsten, Molybdenum, Niobium, Tantalum, Zirconium, Yttrium, Germanium.

13. Method according to claim 9 or 12, wherein after the continuous or discontinuous melting said alloy is subject to a cooling step followed by one or more hot or cold plastic deformation steps and one or more thermal treatments.

14. Item of jewelry, comprising a Copper Gold alloy according to one or more of the preceding claims 1 to 7, wherein said item of jewellery comprises a jewel or watch or bracelet for a watch or a movement or a part of a mechanical movement for a watch.

## Patentansprüche

1. Legierung, insbesondere für Schmuck, **dadurch gekennzeichnet, dass** sie aus:
- Gold, in einer Menge von 330 Gew.-%o bis 420 Gew.-%o;
- Kupfer, in einer Menge von 500 Gew.-%o bis 620 Gew.-%o;
- Palladium, in einer Menge von 5 Gew.-%o bis 35 Gew.-%o;
und gegebenenfalls Eisen in einer Menge von 2 Gew.-%o bis 25 Gew.-%o, vorzugsweise von 5 Gew.-%o bis 20 Gew.-%o, besteht.

2. Legierung nach Anspruch 1, **dadurch gekennzeichnet, dass** sie eine dunkelrote Farbe aufweist und/oder dadurch, dass sie eine Farbe aufweist, die auf der CIELAB1976-Farbkarte eine Koordinate a* > 8,2 und eine Koordinate b* < 13,55 aufweist, wobei die CIELAB1976-Farbkarte eine Farbe auf der Grundlage eines ersten L*-Parameters, eines zweiten a*-Parameters und eines dritten b*-Parameters definiert, wobei der erste L*-Parameter die Helligkeit angibt und Werte, umfasst zwischen 0 für Schwarz und 100 für Weiß, annimmt, während der zweite a*-Parameter und der dritte b*-Parameter Chromatizitätsparameter darstellen, wobei der zweite a*- und dritte b*-Parameter durch die folgenden Formeln in Relation stehen ${C}_{ab} * = \sqrt{\left(a{∗}^{2}+b{∗}^{2}\right)}$ ${h}_{ab ∗} = {tan}^{- 1} \left(\frac{b ∗}{a ∗}\right)$ wobei C_{ab}* als "Chroma" definiert ist und die Farbsättigung angibt, und wobei h_{ab*} die Tonalität der Farbe angibt.

3. Legierung nach einem der vorhergehenden Ansprüche, wobei Palladium in einer Menge von 8 Gew.-%o, vorzugsweise von 10 Gew.-%o, bis 32 Gew.-%o, stärker bevorzugt bis 30 Gew.-%o, vorhanden ist.

4. Legierung nach Anspruch 3, wobei Palladium in einer Menge von 15 Gew.- ‰ bis 25 Gew.-%o, vorzugsweise von 18 Gew.-%o bis 22 Gew.-%o, stärker bevorzugt in einer Menge von im Wesentlichen gleich 20 Gew.-%o, vorhanden ist.

5. Legierung nach einem oder mehreren der vorhergehenden Ansprüche, wobei die Summe der Mengen an Palladium und Eisen gleich 30 Gew.-%o ist.

6. Legierung nach einem der vorhergehenden Ansprüche, wobei Gold in einer Menge von 365 Gew.-‰ bis 385 Gew.-‰ vorhanden ist und Kupfer in einer Menge von 594 Gew.-‰ bis 614 Gew.-‰ vorhanden ist und Palladium in einer Menge von 15 Gew.-‰ bis 25 Gew.-‰, gegebenenfalls in einer Menge von 18 Gew.-‰ bis 22 Gew.-‰, umfasst ist.

7. Legierung nach einem der vorhergehenden Ansprüche, **gekennzeichnet durch** die Abwesenheit von Vanadium und anderen Metallen, die Carbide und Oxide bilden können, insbesondere frei von Magnesium, Silizium, Titan, Wolfram, Molybdän, Niob, Tantal, Zirkonium, Yttrium, Germanium, wobei die Legierung auch frei von Nickel, Kobalt, Arsen und Cadmium ist.

8. Verfahren zur Herstellung einer Kupfer-Gold-Legierung für Schmuck, wobei das Verfahren **dadurch gekennzeichnet ist, dass** es umfasst:
a) einen Schritt des Homogenisierens von:
- Gold, in einer Menge von 330 Gew.-%o bis 420 Gew.-%o;
- Kupfer, in einer Menge von 500 Gew.-%o bis 620 Gew.-%o;
- Palladium, in einer Menge von 5 Gew.-%o bis 35 Gew.-%o;
- und gegebenenfalls Eisen in einer Menge von 2 Gew.-%o bis 25 Gew.-%o, vorzugsweise von 5 Gew.-%o bis 20 Gew.-%o;
um eine Mischung herzustellen; und
b) einen Schritt des Einbringens der Mischung in einen Schmelztopf, und ein anschließendes Schmelzen durch Erhitzen bis zum Schmelzen.

9. Verfahren nach Anspruch 8, wobei das Homogenisieren ein diskontinuierliches Schmelzen ist, umfassend einen Schritt des Gießens, wobei das geschmolzene Material in eine feuerfeste Form gegossen wird und wobei die geschmolzene Legierung eine Legierung ist, die durch die Abwesenheit von Vanadium und anderen Elementen, die Carbide oder Oxide bilden können, gekennzeichnet ist, insbesondere frei von Magnesium, Silizium, Titan, Wolfram, Molybdän, Niob, Tantal, Zirkonium, Yttrium, Germanium.

10. Verfahren nach Anspruch 9, wobei der Schmelztopf einer gasgesteuerten Atmosphäre ausgesetzt wird und insbesondere, zumindest zeitweise, einer Vakuumbedingung ausgesetzt wird.

11. Verfahren nach Anspruch 9 oder 10, wobei der Schmelztopf während des Gießschritts einer kontrollierten Atmosphäre und Drücken, die niedriger als der Umgebungsdruck sind, ausgesetzt wird, und wobei die kontrollierte Atmosphäre ein Inertgas, vorzugsweise Argon, ist oder umfasst und/oder der Druck ein Druck von niedriger als 800 mbar, vorzugsweise niedriger als 700 mbar, ist und/oder wobei das Gas ein reduzierendes Gas, vorzugsweise eine Wasserstoff-Stickstoff-Mischung, ist.

12. Verfahren nach Anspruch 11, wobei das Schmelzen ein kontinuierliches Schmelzen ist, umfassend einen Schritt des Schmelzens und Homogenisierens in einem Graphittopf und einen anschließenden Gießschritt, wobei die geschmolzene Legierung in eine Form aus Graphit gegossen wird und wobei die Legierung eine Legierung aus Metallen ist, die dem Graphit chemisch nicht ähnlich sind und stärker spezifisch, insbesondere zumindest frei von Vanadium, Magnesium, Silizium, Titan, Wolfram, Molybdän, Niob, Tantal, Zirkonium, Yttrium, Germanium.

13. Verfahren nach Anspruch 9 oder 12, wobei die Legierung nach dem kontinuierlichen oder diskontinuierlichen Schmelzen einem Abkühlungsschritt ausgesetzt wird, gefolgt von einem oder mehreren Schritten der plastischen Warm- oder Kaltverformung und von einer oder mehreren thermischen Behandlungen.

14. Schmuckstück, umfassend eine Kupfer-Gold-Legierung nach einem oder mehreren der vorhergehenden Ansprüche 1 bis 7, wobei das Schmuckstück einen Schmuck oder Uhr oder Armband für eine Uhr oder ein Uhrwerk oder einen Teil eines mechanischen Uhrwerks für eine Uhr umfasst.

## Revendications

1. Alliage, en particulier de joaillerie, **caractérisé en ce qu'**il est constitué :
- d'or, en une quantité de 330 ‰ à 420 ‰ en poids ;
- de cuivre, en une quantité de 500 ‰ à 620 ‰ en poids ;
- de palladium, en une quantité de 5 ‰ à 35 ‰ en poids ;
et éventuellement de fer en une quantité de 2 ‰ à 25 ‰ en poids, préférablement de 5 ‰ à 20 ‰ en poids.

2. Alliage selon la revendication 1, **caractérisé en ce qu'**il présente une couleur rouge foncé et/ou **en ce qu'**il présente une couleur qui, sur le diagramme de couleur CIELAB1976, présente une coordonnée a* > 8,2 et une coordonnée b* < 13,55, le diagramme de couleur CIELAB1976 définissant une couleur sur la base d'un premier paramètre L*, d'un second paramètre a* et d'un troisième paramètre b*, le premier paramètre L* identifiant la brillance et adoptant des valeurs comprises entre 0 pour noir et 100 pour blanc, tandis que le second paramètre a* et le troisième paramètre b* représentent des paramètres de chromaticité, lesdits second a* et troisième paramètre b* étant associés par les formules suivantes ${C}_{ab *} = \sqrt{\left(a{∗}^{2}+b{∗}^{2}\right)}$ ${h}_{ab *} = {tan}^{- 1} \left(\frac{b ∗}{a ∗}\right)$ C_{ab*} étant défini comme « chroma » et identifiant la saturation de couleur, et *h_{ab*}* identifiant la tonalité de la couleur.

3. Alliage selon l'une quelconque des revendications précédentes, dans lequel le palladium est présent en une quantité de 8 ‰, préférablement de 10 ‰ en poids, à 32 ‰, plus préférablement à 30 ‰ en poids.

4. Alliage selon la revendication 3, dans lequel le palladium est présent en une quantité de 15 ‰ à 25 ‰ en poids, préférablement de 18 ‰ à 22 ‰ en poids, plus préférablement en une quantité sensiblement égale à 20 ‰ en poids.

5. Alliage selon l'une ou plusieurs des revendications précédentes, dans lequel la somme des quantités de palladium et de fer est égale à 30 ‰ en poids.

6. Alliage selon l'une quelconque des revendications précédentes, dans lequel l'or est présent en une quantité de 365 ‰ à 385 ‰ en poids et le cuivre est présent en une quantité de 594 ‰ à 614 ‰ en poids et le palladium étant compris en une quantité de 15 ‰ à 25 ‰ en poids, éventuellement en une quantité de 18 ‰ à 22 ‰ en poids.

7. Alliage selon l'une quelconque des revendications précédentes, **caractérisé par** l'absence de vanadium, et d'autres métaux capables de créer des carbures et des oxydes, en particulier exempts de magnésium, silicium, titane, tungstène, molybdène, niobium, tantale, zirconium, yttrium, germanium, ledit alliage étant également exempt de nickel, cobalt, arsenic et cadmium.

8. Procédé de production d'un alliage de cuivre-or pour joaillerie ; ledit procédé étant **caractérisé en ce qu'**il comprend :
a) une étape d'homogénéisation :
- d'or, en une quantité de 330 ‰ à 420 ‰ en poids ;
- de cuivre, en une quantité de 500 ‰ à 620 ‰ en poids ;
- de palladium, en une quantité de 5 ‰ à 35 ‰ en poids ;
- et éventuellement de fer en une quantité de 2 ‰ à 25 ‰ en poids, préférablement de 5 ‰ à 20 ‰ en poids ;
pour créer un mélange ; et
b) une étape d'introduction du mélange dans une cuve de fusion, et une fusion ultérieure à travers le chauffage jusqu'à la fusion.

9. Procédé selon la revendication 8, dans lequel ladite homogénéisation est une fusion discontinue, comprenant une étape de coulée, dans lequel le matériau fondu est coulé dans un moule réfractaire et dans lequel ledit alliage fondu est un alliage **caractérisé par** l'absence de vanadium, et d'autres éléments capables de créer des carbures ou des oxydes, en particulier exempts de magnésium, silicium, titane, tungstène, molybdène, niobium, tantale, zirconium, yttrium, germanium.

10. Procédé selon la revendication 9, dans lequel la cuve de fusion est soumise à une atmosphère de gaz contrôlée et en particulier est soumise, au moins temporairement, à une condition de vide.

11. Procédé selon la revendication 9 ou 10, dans lequel durant ladite étape de coulée, ladite cuve de fusion est soumise à une atmosphère contrôlée, et à des pressions inférieures à celles de l'environnement et dans lequel ladite atmosphère contrôlée est ou comprend un gaz inerte, préférablement de l'argon et/ou ladite pression étant une pression inférieure à 800 mbar, préférablement inférieure à 700 mbar et/ou dans lequel ledit gaz est un gaz réducteur, préférablement un mélange d'hydrogène-azote.

12. Procédé selon la revendication 11, dans lequel ladite fusion est une fusion continue, comprenant une étape de fusion et d'homogénéisation dans une cuve en graphite et une étape de coulée ultérieure dans laquelle l'alliage fondu est coulé dans un moule réalisé en graphite et dans lequel ledit alliage est un alliage de métaux chimiquement non semblables au graphite et plus spécifiquement, en particulier au moins exempts de vanadium, magnésium, silicium, titane, tungstène, molybdène, niobium, tantale, zirconium, yttrium, germanium.

13. Procédé selon la revendication 9 ou 12, dans lequel après la fusion continue ou discontinue, ledit alliage est soumis à une étape de refroidissement suivie d'une ou plusieurs étapes de déformation plastique à chaud ou à froid et d'un ou plusieurs traitements thermiques.

14. Article de joaillerie, comprenant un alliage de cuivre-or selon l'une ou plusieurs des revendications précédentes 1 à 7, dans lequel ledit article de joaillerie comprend un bijou ou une montre ou un bracelet pour une montre ou un mouvement ou une partie d'un mouvement mécanique destiné à une montre.
